

Feb. 8, 1949.

F. C. TOETTCHER

2,461,454

MANUFACTURE OF LUBRICATING OIL

Filed May 4, 1945



INVENTOR.  
FRED C. TOETTCHER.

BY

*Daniel Shyler*  
ATTORNEY.

## UNITED STATES PATENT OFFICE

2,461,454

## MANUFACTURE OF LUBRICATING OIL

Fred C. Toettcher, Fishkill, N. Y., assignor to The Texas Company, New York, N. Y., a corporation of Delaware

Application May 4, 1945, Serial No. 592,055

2 Claims. (Cl. 196—147)

1

This invention relates to the catalytic treatment of hydrocarbon oils to produce lubricating oils highly resistant to oxidation. The invention is concerned with certain improvements in the treatment of lubricating stocks to effect improvement in oxidation stability and to produce oils of highly stable character adapted for turbine oils, lubricating oils for internal combustion engines and the like.

In accordance with the invention the oil is fractionated into a plurality of fractions and these fractions or a selected fraction or selected fractions thereof are subjected to catalytic treatment to effect improvement in oxidation stability. The invention is based on the discovery that when lubricating oil is subjected to the catalytic treatment the extent of improvement in oxidation stability is generally greater in the higher boiling or higher viscosity components of the treated product and that when an oil stock is fractionated into a plurality of cuts and the several cuts subjected to separate catalytic treatments of identical severity greater improvement in oxidation stability is produced on the higher boiling or higher viscosity fractions.

For the purpose of fully disclosing the invention reference is had to the accompanying drawing which is a graph showing a comparison of the treatment of the entire stock with the treatment of separated fractions thereof.

In order to show the advantages of the invention a comparison is made between the catalytic treatment of the entire stock and the treatment of certain fractions thereof. A naphthenic pale oil stock of 500/100° F. Saybolt Universal viscosity was subjected to fractionation under vacuum distillation to produce 10% distillate cuts and a residual or bottoms fraction. Certain of these fractions including the 20-30%, the 40-50%, the 60-70%, the 80-90% fractions of the distillate and the undistilled bottoms were each separately treated with Super Filtral (10% by weight) at 600° F. for a period of one and one-half hours. In the drawing the 10% fractions and the bottoms fraction are plotted as abscissa and the oxidation stability as determined by the A. S. T. M. Turbine Oil Oxidation test is plotted as ordinates (the test life is expressed as the number of hours required for the oil to reach a neutralization number of 2). Curve A or the dots thereon indicate the oxidation test life of the several products obtained in the catalytic treatment of the several fractions of the pale oil. Each of the catalytically treated products was subjected to distillation to strip off a light fraction constituting

2

10% of the treated product. Curve B or the points thereon (solid triangles) indicate the oxidation test life of the stripped products. It will be observed that the stripped products have considerably longer test life than the unstripped products. The entire pale oil stock was also subjected to catalytic treatment under the same conditions as were applied to the several fractions and the resultant product was fractionated to obtain 10% distillate cuts and a residual or bottoms fraction. Curve C or the points thereon (open triangles) represent the oxidation test life of these fractions.

It is evident from the data that considerably longer oxidation test life can be obtained by the catalytic treatment of the fractions than by treating the whole oil stock in one operation. Accordingly in practicing the invention the lubricating stock is fractionated into a plurality of cuts and each of these cuts or selected cuts are subjected to the catalytic cracking. The several products, preferably after stripping off the lighter fractions, are then blended to produce a high quality lubricating oil. The fractionation of the lubricating oil to obtain the fractions for treatment and the stripping of the treated fractions are preferably conducted under vacuum distillation so as to avoid thermal cracking. In the stripping of the treated products the distillation may be conducted to an extent sufficient to reduce each treated fraction to the same viscosity as that of the fraction before the catalytic treatment or each treated fraction may be stripped to yield a product of even higher viscosity than such fraction.

35 The catalysts which are adapted for the practice of the invention comprise certain composites of silica and alumina and include generally the activable clays particularly the non-swelling, acid treated montmorillonite or bentonitic clays. Industrial clays which have been found particularly effective are Super Filtral and Lena clay each of which is a non-swelling, acid treated bentonitic clay.

In the treatment to effect the increase in oxidation stability the lubricating stock is contacted with the catalyst in pulverulent, comminuted form at temperatures upwards of 600° F. In order to obtain the maximum improvement in oxidation stability without undue loss in product, due to conversion into lower boiling products than desired for the lubricating oil product, the most satisfactory temperature is within a range of about 650-725° F. with a period of reaction of about one-half an hour up to one or two hours. It is desirable that the treatment be conducted

with the oil essentially in the liquid phase and consequently the temperature should be kept below the critical temperature of the stock being treated. Moreover, as the temperature is increased there is greater danger of having thermal cracking at the expense of the desired selective catalytic conversion. Consequently in order to avoid cracking into low boiling components, such as gasoline, the upper limit of the temperature of treatment for the lubricating oil stocks is about 750° and generally a temperature of about 650-725° F. is the most satisfactory. For the most effective operation the quantity of catalyst used should be about 8-10% by weight of the oil treated or greater proportions up to around 20%.

Under these conditions the catalyst promotes reactions in which the structures of the lubricating oil molecules which are relatively unstable to oxidation are modified to more stable structures, structures which inhibit the oxidation of lubricating oil or to structures which may readily be removed from the oil by simple methods such, for example, as distillation. While it is difficult to determine the exact nature of the reactions in the treatment, it appears that in general there is some increase in both aromaticity and paraffinicity apparently at the expense of naphthenic rings.

In accordance with the invention the lubricating oil is fractionated into a plurality of cuts and the several fractions or selected fractions thereof, especially the higher viscosity fractions, are separately subjected to the catalytic conversion to effect increase in oxidation stability. In one method of operation the less viscous fractions may be subjected to more drastic conversion conditions than the higher viscosity fractions. The several treated products are stripped to produce products of the same or higher viscosity as that of the fractions before the treatment and the stripped products are blended with the untreated fractions to produce a composite product of desired viscosity and oxidation stability. In one method of operation the lubricating stock is fractionated to produce a single fraction for catalytic treatment such for example, as a 10% to 25% fraction comprising the higher boiling components of the stock; this fraction is subjected to the catalytic treatment and stripped deeply to produce a high concentration of the stabilizing components and this stripped product is blended with the untreated portion of the original stock. Generally it is considered more satisfactory to apply the catalytic conversion to one or more relatively narrow fractions having a viscosity or viscosities above that of the viscosity desired for the final blended product.

In one method of operation in accordance with the invention, lower boiling fractions obtained in the fractionation of the catalytically treated products, more particularly the fractions of lower viscosity than that of the charge to the catalytic treating operation, may be recycled to the catalytic treating zone so that the lower viscosity constituents may thus be subjected to further conversion for increase in oxidation stability.

The invention is adapted for the treatment of either raw lubricating stocks or refined stocks in so far as effecting the improvement in oxidation stability is concerned. However in the treatment of oils for certain purposes as in the production of turbine oils which are required to have a high oxidation stability and also must be resistant to emulsion or must readily separate from emulsions which may be produced in the use of

the oil, it is necessary that the catalytic treatment be applied after the oil has been subjected to the refining treatment, such as acid treatment and solvent refining, since if the oil, after being given the catalytic treatment, be subjected to after-treatments, such as sulfuric acid treating, solvent refining, caustic washing and similar treatments, while the emulsion characteristics of the oil may be improved the after-treating tends to greatly reduce the oxidation stability imparted to the oil by the catalytic treatment. Accordingly in the production of an oil which will have both high oxidation stability and good emulsion characteristics, it is critical that the catalytic treatment for improvement in oxidation stability follow the other refining treatments. The catalytically treated oil or the blend of the catalytically and untreated oil may further be subjected to filtration through clay or fuller's earth at moderate temperature for improvement in color without impairing its quality for turbine oils.

In practicing the invention the mixture of oil and catalysts may be subjected to reaction in various types of apparatus. A preferred operation is to pass the mixture of oil and comminuted catalyst through a carefully regulated heating coil and to either quench the effluent or to pass it through a cooler adapted for rapid cooling so as to thus accurately control the time of reaction. The catalyst should be added to the oil with the oil at normal temperature or at least after only moderate preheating so as to eliminate the effect of any strictly thermal reaction. The cooled oil is passed to a distilling or fractionating zone for removing the lighter fractions. These lighter fractions may be removed from the system or recycled to the heating coil. A plurality of heating and fractionating units may be employed so as to simultaneously treat the various fractions.

Although a preferred embodiment of the invention has been described herein, it will be understood that various changes and modifications may be made therein, while securing to a greater or less extent some or all of the benefits of the invention, without departing from the spirit and scope thereof.

I claim:

1. The method of improving the oxidation stability of lubricating oil of the pale oil type that comprises separating from the lubricating oil a minor fraction constituting the higher boiling portion thereof, treating the minor fraction with activated clay at a temperature upwards of 600° F. and not in excess of about 750° F. with a reaction time of the order of  $\frac{1}{2}$ -2 hours to thereby effect reactions involving an increase in aromaticity and formation of structures which inhibit oxidation, distilling off lower boiling constituents from the treated fraction to thereby concentrate the oxidation inhibiting constituents and blending the resultant stripped product with the untreated major portion of the lubricating oil to produce a blended product of increased oxidation stability.
2. The method of improving the oxidation stability of lubricating oil of the pale oil type that comprises separating from the lubricating oil a higher boiling fraction thereof constituting about 10-25% of the oil, treating said fraction with activated clay at a temperature upwards of 600° F. and not in excess of about 750° F. with a reaction time of the order of  $\frac{1}{2}$ -2 hours to thereby effect reactions involving an increase in aromaticity and formation of structures which inhibit oxidation, distilling off lower boiling con-

stituents from the treated fraction to thereby concentrate the oxidation inhibiting constituents and blending the resultant stripped product with the untreated major portion of the lubricating oil to produce a blended product of increased 5 oxidation stability.

FRED C. TOETTCHER.

REFERENCES CITED

The following references are of record in the 10 file of this patent:

UNITED STATES PATENTS

| Number    | Name     | Date          | Number | Name      | Date |
|-----------|----------|---------------|--------|-----------|------|
| 1,547,682 | Puitzman | July 28, 1925 | 15     | 2,356,952 |      |
| 1,655,175 | Benjamin | Jan. 3, 1928  |        | 2,420,108 |      |

| Name              | Date          |
|-------------------|---------------|
| Johnston          | June 24, 1930 |
| Isom et al.       | Dec. 30, 1930 |
| Lowery et al.     | July 7, 1931  |
| Stafford          | May 3, 1932   |
| Darlington        | Oct. 25, 1932 |
| Belden            | Feb. 21, 1933 |
| Beiswenger        | Aug. 21, 1934 |
| Tuttle            | Feb. 9, 1937  |
| Brandt            | Nov. 19, 1940 |
| Bray et al        | July 1, 1941  |
| Schumacher et al. | Feb. 17, 1942 |
| Evans et al.      | Feb. 8, 1944  |
| Lovell            | Feb. 15, 1944 |
| Smith             | Aug. 29, 1944 |
| Stratford et al.  | May 6, 1947   |

**Certificate of Correction**

Patent No. 2,461,454.

February 8, 1949.

**FRED C. TOETTCHER**

It is hereby certified that error appears in the printed specification of the above numbered patent requiring correction as follows:

Column 2, line 46, after the word "communited" insert *or powdered*;  
and that the said Letters Patent should be read with this correction therein that the same may conform to the record of the case in the Patent Office.

Signed and sealed this 7th day of June, A. D. 1949.

[~~SEAL~~]

**THOMAS F. MURPHY,**  
*Assistant Commissioner of Patents.*